

F. HAUPTMEYER.

MATERIAL FOR ARTIFICIAL INTERNAL MEMBERS OF THE HUMAN BODY.  
APPLICATION FILED SEPT. 3, 1920.

1,421,776.

Patented July 4, 1922.



Inventor

Friedrich Hauptmeyer,

By

*Knight Bros.*

Attorneys

# UNITED STATES PATENT OFFICE.

FRIEDRICH HAUPTMEYER, OF ESSEN, GERMANY.

## MATERIAL FOR ARTIFICIAL INTERNAL MEMBERS OF THE HUMAN BODY.

1,421,776.

Specification of Letters Patent. Patented July 4, 1922.

Application filed September 3, 1920. Serial No. 408,083.

To all whom it may concern:

Be it known that Dr. FRIEDRICH HAUPTMEYER, a citizen of Germany, residing at Essen, Germany, has invented certain new and useful Improvements in Material for Artificial Internal Members of the Human Body, of which the following is a specification.

The invention refers to artificial members to be used internally for human or animal organisms, in particular to supports for teeth and means for fastening the teeth to said supports and consists in employing for the manufacture of said artificial members a chromium-nickel-steel alloy containing about 18 to 23 per cent chromium, 5 to 10 per cent nickel and 0.1 to 0.4 per cent carbon. These alloys which resist oxidizing and deteriorating influences of the organism practically to the same degree as precious metals such as platinum, gold and silver, but which are considerably cheaper than the latter, are capable not only to form substitutes of these precious metals, but they surpass them in many respects.

The tensile strength and hardness of chromium-nickel-steel, both of which are throughout greater than those of precious metals, render it possible to construct artificial bone portions, mouth plates and other elements of artificial sets of teeth as well as orthodontic apparatus for internal adaptation very light without impairing their strength and durability. This is a considerable advantage over precious metals whose scarcity and high price has in many instances caused too light a construction of the artificial members to render them durable. Moreover the use of chromium-nickel-steel alloys of the character described has the further advantage that owing to their comparatively small value, no regard need be taken of the waste which occurs during manufacturing so that the manufacturing methods may be materially simplified.

It is also important that chromium-nickel-steel alloys of this character when used in artificial sets of teeth have no taste and further that their expansion coefficient is equal to that of the kind of porcelain

which is used for artificial teeth. Thus for instance, when chromium-nickel-steel pins are burned into the porcelain crowns of teeth, the latter are not cracked and split by undue expansion of the pins.

Furthermore, chromium-nickel-steel alloys when attached to artificial teeth by burning processes or the like, will not discolor the porcelain which is otherwise the case with every metal except platinum.

The annexed drawing shows for illustration, an upper plate in section, the palate part *a* of which together with the hook *b* is made of the alloy of the specified character. The fastening pins *c* connecting the porcelain front *d* of the teeth with the palate part *a* are also made of this alloy.

### Claims.

1. As a new article of manufacture a porcelain tooth element, a supporting structure for said element and a connecting chromium-nickel-steel pin for attaching said porcelain element to said structure, said pin having the composition chromium 18 to 23 per cent, nickel 5 to 10 per cent, carbon .1 to .4 per cent.

2. A new article of manufacture comprising a porcelain tooth element having a burnt-in chromium-nickel-steel pin of the composition chromium 18 to 23 per cent, nickel 5 to 10 per cent, carbon .1 to .4 per cent.

3. In combination with a tooth, a dental support for said tooth, said support made up of the physiologically inert chromium-nickel-steel alloy, having the composition chromium 18 to 23 per cent, nickel 5 to 10 per cent, carbon .1 to .4 per cent.

4. As a new article of manufacture a porcelain crown element having a burnt-in chromium-nickel-steel pin of the composition chromium 18 to 23 per cent, nickel 5 to 10 per cent, carbon .1 to .4 per cent.

5. As a new article of manufacture, an artificial member to be used internally for living organisms made up of a chromium-nickel-steel alloy having the composition chromium 18 to 23 per cent, nickel 5 to 10 per cent, carbon .1 to .4 per cent.

FRIEDRICH HAUPTMEYER.